

Patented June 4, 1929.

1,716,050

# UNITED STATES PATENT OFFICE.

WILLIAM M. GROSVENOR AND VICTOR P. GERSHON, OF NEW YORK, N. Y.; SAID GERSHON ASSIGNOR TO SAID GROSVENOR.

## MANUFACTURE OF ALLOYS.

No Drawing.

Application filed February 3, 1925. Serial No. 6,540.

Our invention relates to improvements in the manufacture of alloys and more particularly to base alloys adapted for the manufacture of white gold and the method of 5 making white gold therewith. As is known in the art, white gold is an alloy of gold, nickel and zinc, some containing also one or more other metals such as copper or palladium. White gold was formerly made 10 by melting for example 15 parts gold and adding to the molten gold and melting therein 4 parts of nickel and 1 part of zinc by weight, the whole being covered with a suitable flux. The main difficulty with 15 this method was that, in spite of the flux, more or less zinc is volatilized and lost so that the resulting alloy is variable and such variations, particularly in respect of the quantity of zinc result in an inferior if not 20 useless gold alloy, and only in the hands of skilled manufacturers of alloys is it possible to obtain commercial results, and even then such alloys often contain oxides produced by the oxygen from the air of hydrogen compounds caused by the action of 25 hydrogen from the moisture of the air, which render the alloy excessively brittle. Therefore, the process is not well adapted for the average jeweller to carry out. Most jewelers, furthermore, prefer to make up their 30 own gold, because the gold they require varies as to number of karats and by making up their own white gold from fine gold and base metal they can get any karat gold 35 they desire and do not have to carry in stock substantial quantities of made up gold of different karats involving relatively large carrying charges. To meet this demand of the jewellers, attempts have been made to 40 supply the jewellers with base metals or alloys which the jewellers might readily alloy with fine gold in any desired proportion. The desideratum has been a base alloy containing nickel and zinc in proportions to make white gold. In the first mentioned method of making white gold by adding the unalloyed nickel and zinc to the molten gold, it is known that the zinc should 45 be about one fifth of the base metal, e. g. if nickel and zinc alone are used to form the base metal to be alloyed with the fine gold, 4 parts of nickel to 1 part by weight of zinc 50 would be used, and if for example it were desired to produce an 18 karat white gold, 55 4 parts nickel and 1 part zinc and 15 parts of fine gold would be used. A base alloy of about 80% nickel and 20% zinc suitable to be thus alloyed with gold, has not, so far as we are aware, been heretofore produced. It is well known that zinc boils and vaporizes at a temperature well below the melting point of nickel and if nickel be added to molten zinc it is found that only a relatively small percentage of the nickel will be taken up, while if zinc be added to molten 60 nickel or the two heated together to a temperature sufficient to melt them, a large part of the zinc volatilizes making it impossible to obtain a resulting nickel-zinc alloy of predetermined composition of anything like the 65 80-20 proportion, which must be quite closely adhered to in so far as the proportion of zinc is concerned if a satisfactory white gold is to be obtained.

To obtain an alloy which jewellers might 70 melt up with gold to make such white gold, it has been suggested that an alloy containing the zinc and about equal parts of copper and nickel be used. This base alloy contained over 40% copper. By using this 75 copper it was found that over 15% and about 10% of nickel of zinc could be gotten in the resulting base alloy of nickel, copper and zinc. When, however, this base alloy was melted with fine gold to make 18 karat 80 or other usual karat white gold, it was found that the resulting gold was tinged with yellow or red and off color and did not have that desirable whiteness substantially 85 like that of platinum.

To avoid this and reduce the amount of copper in the resulting gold it has been suggested that two metals be furnished the jewellers, one being merely nickel and the other an alloy of copper and zinc with or 90 without a small amount of nickel and/or palladium. In this way the amount of copper introduced into the final gold has been reduced to about 10% of the base metal, whereby the resulting gold is of much better 95 color. This method has the disadvantage however, that the base metals must be carefully weighed out (as well as the gold) and a mistake in weighing out either of the two base metals is likely to result in a substantial 100 change in the proportion of zinc in the resulting alloy which in turn will result in an inferior white gold if not a useless alloy. Likewise mistakes are frequently made by 105 interchanging one base metal or alloy for 110

another. Also there is danger of loss of zinc by volatilization. The method is therefore not only inconvenient but quite difficult of manipulation, uncertain in result, and a single base alloy suitable for melting with fine gold in proportions to make 18 or other usual karat gold has been long sought.

Accordingly in our copending application for U. S. Letters Patent Ser. No. 6539, filed February 3, 1925, now Patent 1,688,642, granted May 8, 1928, we have described a new base metal comprising a substantially uniform and homogeneous alloy containing nickel and zinc or a material containing nickel and zinc alloyed together, the zinc being about 20% of the alloy or material and the nickel about 80%, the alloy or material having the characteristic that when melted and alloyed, for example, with 3 times its weight of fine gold, the resultant gold alloy not only exhibits a whiteness substantially like that of platinum but it is also capable of being cast and rolled for making jewelry. In that application we further disclosed that such a base alloy containing about 20% of zinc can be produced by melting the zinc and nickel under pressure whereby the volatilization of the zinc is prevented so that alloys of nickel and zinc and containing a substantially accurate predetermined percentage of zinc can be satisfactorily obtained.

While such base alloy is well adapted for the making of white gold as above explained, we have further discovered that the base alloy is much improved if small amounts of certain other metals are included therein such as copper and/or a small amount of gold. By including in the base alloy a small amount of other metal such as about 9% copper, we find that the base alloy may be made under pressures considerably lower than would otherwise be the case. The addition of the small amount of copper in the base alloy results in a base alloy which when alloyed with fine gold in proportion to make 18 karat or other usual proportion white gold, results in a white gold which is still better adapted for die stamping and draw-pressing than when copper is not used. The qualities of the resulting white gold with respect to rolling, casting, die stamping, etc., we find are also improved if a small quantity of gold be included in the base alloy and for this purpose we prefer to add about 1% or less of fine gold. If desired the copper may be omitted and only the gold included with the nickel and zinc or vice versa depending on the use to

which the resulting white gold is to be put, but we prefer to include both the copper and gold in the base alloy.

To form the base alloy the nickel, zinc, copper and gold, in suitable small pieces and in the proper proportions, are preferably placed in an electric furnace and the mixture melted under pressure to prevent the volatilization of the zinc. A pressure considerably under 15 atmospheres (for instance 6 or less) will usually be found sufficient. Also the alloying should be carried out in an inert atmosphere preferably an atmosphere of nitrogen, all as described in our said copending application, and preferably with an apparatus such as described in our said copending application.

The resulting base alloy may be readily alloyed with 3 times its weight of fine gold to make 18 karat gold or any usual proportion and this is easily done by the various jewelers in a manner with which they are accustomed. The resultant gold alloy not only exhibits a whiteness substantially like that of platinum but it is also capable of being readily cast, rolled and stamped for making many kinds of jewelry.

The resultant white gold is also well adapted for draw-pressing.

While we have described our improvements in great detail and in connection with a preferred embodiment thereof, we do not desire to be limited to such details or embodiments since many changes and modifications may be made and the invention embodied in widely different forms without departing from the spirit and scope of the improvements in their broader aspects. Hence we desire to cover all modifications and forms coming within the language or scope of any one or more of the appended claims.

What we claim as new and desire to secure by Letters Patent is:

1. A material containing zinc, nickel and copper alloyed together, the material containing about 20% of zinc, about 70% or more of nickel and copper in any amount up to 9%.

2. An alloy material containing zinc, nickel, copper and gold alloyed together, the material containing about 20% of zinc, about 70% or more of nickel, copper in any amount up to 9%, and gold.

3. An alloy containing about 20% of zinc, about 9% of copper, about 1% of gold and about 70% of nickel.

In testimony whereof we have signed our names to this specification.

WILLIAM M. GROSVENOR.  
VICTOR P. GERSHON.